

Aug. 7, 1928.

1,679,435

J. McFETRIDGE

## MANUFACTURE OF METALLIC COATED SHEETS AND PLATES

Filed Jan. 17, 1927

2 Sheets-Sheet 1



*Witnesses:*

Edwin Trueb

*Inventor:*

JOSEPH MCFETRIDGE,

by: JOSEPH H. TREDGE,  
Anthony Usina  
his Attorney

Aug. 7, 1928.

1,679,435

J. McFETRIDGE

MANUFACTURE OF METALLIC COATED SHEETS AND PLATES

Filed Jan. 17, 1927

2 Sheets-Sheet 2

Fig. 1<sup>a</sup>.



Witnesses:

Edwin Trueb

by:

Inventor:

JOSEPH McFETRIDGE,

Anthony Usina  
his Attorney.

## UNITED STATES PATENT OFFICE.

JOSEPH MCFETRIDGE, OF VANDERGRIFT, PENNSYLVANIA, ASSIGNOR TO AMERICAN SHEET AND TIN PLATE COMPANY, OF PITTSBURGH, PENNSYLVANIA, A CORPORATION OF NEW JERSEY.

## MANUFACTURE OF METALLIC-COATED SHEETS AND PLATES.

Application filed January 17, 1927. Serial No. 161,634.

This invention relates to the manufacture of metallic coated sheets and plates, and more particularly to an improved method and apparatus for preparing sheets and plates for galvanizing, tinning and the like, and has for one of its objects the provision of a method for treating the sheets and plates which will prevent rapid oxidation of the sheets and plates to ferric form 10 after pickling.

Another object is to provide a method wherein the sheets and plates may be cleaned by passing through a diluted solution of sulfuric acid prior to being passed into the 15 flux side of the coating pot, instead of being passed through a hydrochloric acid bath which is much more expensive than sulfuric acid.

A further object is to provide a novel 20 method whereby the sheets will carry liquid flux into the flux side of the coating pot to maintain a constant body of flux in the pot.

A still further object is to provide a novel 25 form of apparatus for carrying out my novel method described and claimed herein.

Heretofore the usual practice in preparing sheets and plates for galvanizing, tinning and the like, has been to place from fifty to 30 several hundred sheets, depending upon the gage and size of the sheets, side by side in a rack, then submerge the rack containing the sheets in a hot acid bath. After the sheets have been cleaned or pickled, the rack 35 containing the sheets is removed from the acid bath and immediately submerged in a tank of cold running water, for the purpose of removing the free acid and soluble iron salts from the sheets.

40 At best the above method provided imperfectly cleaned and washed sheets, and the surface of such sheets rapidly oxidized to the ferric form which materially increased the cost of the subsequent treatment steps.

45 After the sheets were washed as described above, they were submerged in a bath of diluted hydrochloric acid, and then passed into the flux side of the coating pot. In this 50 last operation the ferric hydroxide on the sheets was only partly removed, so that the sheets entered the coating pot with ferric hydroxide still on their surfaces. Hereto-

fore ammonia chloride crystals have been added from time to time to the flux in the 55 coating pot to maintain the flux in active condition. The imperfectly washed sheets resulting from the method described above are entered into the flux side of the coating pot covered with a solution of diluted 60 hydrochloric acid, ferrous chlorid and ferric hydroxide. The ferric hydroxide and soluble iron salts entering the flux, are removed in the flux and the iron combines with coating material or metal to form an alloy, 65 which in galvanizing is called zinc dross since it is an alloy of zinc and iron.

The present method consists in part in completely cleaning or pickling the sheets and plates by submersion in a hot pickle or 70 acid bath, then submerging the cleaned or pickled sheets or plates in a cold solution of inorganic salts until cooled to approximately 100 degrees Fahrenheit or less, then removing the sheets and plates from the inorganic 75 salt solution. The sheets and plates treated as above may be stored a reasonable length of time without the formation of ferric hydroxide, or, if such sheets are exposed separately, the sheets or plates will dry from 80 the heat absorbed from the hot pickle liquor, and a film of ferrous salts will form on the sheets so as to provide a protective coating, whereby the sheets or plates may be stored for hours without the formation of ferric 85 hydroxide.

After the sheets or plates have been cleaned and immersed in the cold solution of soluble inorganic salts, the sheets are next passed through a diluted sulfuric acid bath 90 having a strength of from 5 degrees Bé. to 15 degrees Bé., to remove any ferrous hydroxide that may be formed thereon, and the finally cleaned plates are then passed between suitable sprays of either hot or cold 95 water which thoroughly wash both sides of the sheets or plates to remove all acid and soluble iron salts. The sheets and plates when they pass between the washing sprays, they are free from all solid foreign matter, 100 but are wet with diluted sulfuric acid and soluble iron salts, all of which are removed or washed off by the water sprays. After the sheets pass between the water sprays and are washed, they are then passed into 105 a flux tank containing a body of liquid flux,

such as a solution of ammonia chlorid, zinc chlorid, zinc ammonia chlorid, and the like, heated to from 160 to 180 degrees Fahrenheit. The sheets as they pass through the flux in the flux tank are wetted with the flux and also preheated by the heated flux and are then passed directly into the flux side of the coating pot, and the sheets due to being wetted with flux from the flux tank will carry sufficient flux over into the flux side of the coating pot to replenish the supply of flux in the coating pot.

The cold solution of inorganic salts in which the sheets or plates are immersed or submerged immediately after pickling and without washing, may consist of cold spent pickle liquor (ferrous sulfate), zinc chlorid, zinc or sodium sulfate, or other chlorids and sulfates, and the term inorganic salts as used throughout this specification and claims is used to define the above mentioned salts.

In the drawings—

Figures 1 and 1<sup>a</sup> show a longitudinal sectional elevation through apparatus used in carrying out the steps of the method subsequent to the removal of the plates from the solution of inorganic salts.

Figure 2 is a transverse sectional elevation 30 through the washing tank taken on the line II—II of Figure 1.

In carrying out this invention in practice the sheets or plates after being pickled and cooled in the cold solution of inorganic salts, such as the cold spent pickle liquor (ferrous sulfate), or other sulfates and chlorids, are removed from the bath of inorganic salts, and piled or stacked on a transfer wagon or truck A to be transferred to the location of the remainder of the apparatus necessary to carry out the remaining steps of the invention.

The transfer wagon A, after being loaded with sheets or plates B from the inorganic salt bath, is moved into position to have its load fed into the bite of a pair of feed rolls 2 mounted at the entrance end of an acid bath tank 3 which is preferably filled with a bath of diluted sulfuric acid.

The sheets or plates B will be manually or otherwise fed from the truck A into the bite of the feed rolls 2 and the rolls 2 will feed the plates between guides 4, which will guide the plates or sheets down through the acid bath and up into the bite of a pair of feed rolls 5 mounted between the acid bath tank 3 and a washing or spraying space 6.

A pair of horizontally arranged and spaced sprays 7 are mounted in the tank 6 and a guide support or rack, composed of spaced bars 8, is arranged to guide the sheets or plates between the sprays 7 so that both top and bottom sides of the plates will be thoroughly washed.

The rolls 5 will feed the sheets or plates

from the tank 3 along the guide rack composed of bars 8, between the sprays 7 and into the bite of a third pair of feed rolls 10, which are mounted between wash tank 6 and a flux tank 12.

The flux tank 12 is normally filled with a liquid flux, such as a solution of ammonia chlorid, or zinc ammonia chlorid, and is provided with spaced guides 13 for guiding the plates or sheets through the flux and into the bite of a pair of feed rolls 14.

The feed rolls 10 are adapted to feed the sheets or plates through the flux tank and into the bite of the feed rolls 14, which in turn feed the sheets or plates into the bite of feed rolls 16 on the flux side X of a coating pot Y of standard design.

The plates as they pass through and from the flux in the tank 12, will pick up and carry sufficient liquid flux to maintain the body of flux in the flux side of the coating pot Y constant, thereby eliminating the necessity of adding flux in crystal form to the flux in the flux side of the coating pot, which practice results in from forty to fifty per cent. of the added flux being lost through volatilization.

While I have described a certain specific arrangement of the steps of my novel method and certain specific apparatus for carrying out part of such method, it will be understood that I do not wish to be limited thereto, since various modifications may be made without departing from the scope of my invention as defined in the appended claims.

I claim—

1. The method of preparing sheets and plates for galvanizing, tinning and the like, including the step of removing the sheets and plates from the hot pickle bath and without washing submerging said sheets and plates in a cold solution of soluble inorganic salts.

2. The method of preparing sheets and plates for galvanizing, tinning and the like, including the step of removing the sheets and plates from the hot pickle bath and without washing submerging said sheets and plates in cold spent pickle liquor.

3. The method of preparing sheets and plates for galvanizing, tinning and the like, including the following steps, submerging the sheets and plates in a hot acid pickling bath, removing said sheets and plates from said pickling bath and without washing submerging said sheets and plates in a cold solution of soluble inorganic salts, and holding said sheets and plates in said solution of soluble inorganic salts until said sheets and plates are cooled to approximately 100 degrees Fahrenheit.

4. The method of preparing sheets and plates for galvanizing, tinning and the like, including the following steps, submerging

- the sheets and plates in a hot acid pickling bath, removing said sheets and plates from said pickling bath and without washing submerging said sheets and plates in a cold spent pickle liquor bath, and holding said sheets and plates in said cold spent pickle liquor bath until said sheets and plates are cooled to approximately 100 degrees Fahrenheit.
10. 5. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then submerging said sheets and plates in an acid solution to remove any ferrous hydroxide, then washing said sheets and plates to remove all soluble ferrous salts, and then passing said washed sheets and plates immediately through a body of flux prior to entering said sheets and plates into the flux side of the coating pot.
15. 6. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then submerging said sheets and plates in an acid solution to remove any ferrous hydroxide, then washing said sheets and plates to remove all soluble ferrous salts, and then passing said washed sheets and plates immediately through a body of flux prior to entering said sheets and plates into the flux side of the coating pot.
20. 7. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then submerging said sheets and plates in an acid solution to remove any ferrous hydroxide, then washing said sheets and plates to remove all soluble ferrous salts, and then passing said washed sheets and plates immediately through a body of flux prior to entering said sheets and plates into the flux side of the coating pot.
25. 8. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then submerging said sheets and plates in a sulfuric acid solution to remove any ferrous hydroxide, then spraying both sides of said sheets and plates to remove all soluble ferrous salts, and then passing said washed sheets and plates immediately through a body of liquid flux prior to entering said sheets and plates into the flux side of the coating pot.
30. 9. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then submerging said sheets and plates in an acid solution to remove any ferrous hydroxide, then spraying both sides of said sheets and plates to remove all soluble ferrous salts, and then passing said washed sheets and plates immediately through a body of liquid flux prior to entering said sheets and plates into the flux side of the coating pot.
35. 10. The method of preparing sheets and plates for galvanizing, tinning and the like, consisting of submerging the sheets and plates in a hot acid pickling bath, removing said sheets and plates from said pickling bath and without washing submerging said sheets and plates in a cold bath of spent pickle liquor, holding said sheets and plates in said bath until said sheets and plates are cooled to approximately 100 degrees Fahrenheit, removing said sheets and plates from said solution of soluble inorganic salts, then submerging said sheets and plates in an acid solution to remove any ferrous hydroxide, then washing said sheets and plates to remove all soluble ferrous salts, and then passing said washed sheets and plates

immediately through a body of flux prior to entering said sheets and plates into the flux side of the coating pot.

11. The method of preparing sheets and plates for galvanizing, tinning and the like, consisting of submerging the sheets and plates in a hot acid pickling bath, removing said sheets and plates from said pickling bath and without washing submerging said sheets and plates in a cold bath of spent pickle liquor, holding said sheets and plates in said bath until said sheets and plates are cooled to approximately 100 degrees Fahrenheit, removing said sheets and plates from said bath, then submerging said sheets and plates in an acid solution to remove any ferrous hydroxide, then washing said sheets and plates to remove all soluble ferrous salts, and then passing said washed sheets and plates immediately through a body of liquid flux prior to entering said sheets and plates into the flux side of the coating pot, whereby said sheets and plates will carry a quantity of flux from said liquid flux body into the flux on the flux side of said coating pot.

12. The method of preparing sheets and plates for galvanizing, tinning and the like, consisting of submerging the sheets and plates in a hot acid pickling bath, removing said sheets and plates from said pickling bath and without washing submerging said sheets and plates in a cold bath of spent pickle liquor, holding said sheets and plates in said bath until said sheets and plates are cooled to approximately 100 degrees Fahrenheit, removing said sheets and plates from said bath, then submerging said sheets and plates in a sulfuric acid solution to remove any ferrous hydroxide, then washing said sheets and plates to remove all soluble ferrous salts, and then passing said washed sheets and plates immediately through a body of liquid flux prior to entering said sheets and plates into the flux on the flux side of the coating pot, whereby said sheets and plates will carry a quantity of flux from said liquid flux body into the flux on the flux side of said coating pot.

13. The method of preparing sheets and plates for galvanizing, tinning and the like, consisting of submerging the sheets and plates in a hot acid pickling bath, removing said sheets and plates from said pickling bath and without washing submerging said sheets and plates in a cold bath of spent pickle liquor, holding said sheets and plates in said bath until said sheets and plates are cooled to approximately 100 degrees Fahrenheit, removing said sheets and plates from said bath, then submerging said sheets and plates in a sul-

furic acid solution to remove any ferrous hydroxide, then spraying both sides of said sheets and plates to remove all soluble ferrous salts, and then passing said washed sheets and plates immediately through a body of liquid flux prior to entering said sheets and plates into the flux on the flux side of the coating pot, whereby said sheets and plates will carry a quantity of flux from said liquid flux body into the flux on the flux side of said coating pot.

14. The method of preparing sheets and plates for galvanizing, tinning and the like, consisting of submerging the sheets and plates in a hot acid pickling bath, removing said sheets and plates from said pickling bath and without washing submerging said sheets and plates in a cold solution of soluble inorganic salts, holding said sheets and plates in said solution of soluble inorganic salts until said sheets and plates are cooled to approximately 100 degrees Fahrenheit, removing said sheets and plates from said solution of soluble inorganic salts, then exposing said sheets and plates separately to permit said sheets and plates to dry and form a protective coating of ferrous salts thereon, then submerging said sheets and plates in an acid solution to remove any ferrous hydroxide, then washing said sheets and plates to remove all soluble ferrous salts, and then passing said washed sheets and plates immediately through a body of flux prior to entering said sheets and plates into the flux side of the coating pot.

15. The method of preparing sheets and plates for galvanizing, tinning and the like, consisting of submerging the sheets and plates in a hot acid pickling bath, removing said sheets and plates from said pickling bath and without washing submerging said sheets and plates in a cold bath of spent pickle liquor, holding said sheets and plates in said bath until said sheets and plates are cooled to approximately 100 degrees Fahrenheit, removing said sheets and plates from said bath, then exposing said sheets and plates separately to permit said sheets and plates to dry and form a protective coating of ferrous salts thereon, then submerging said sheets and plates in an acid solution to remove any ferrous hydroxide, then washing said sheets and plates to remove all soluble ferrous salts, and then passing said washed sheets and plates immediately through a body of flux prior to entering said sheets and plates into the flux side of the coating pot.

In testimony whereof, I have hereunto signed my name.

JOSEPH McFETRIDGE.